

# UNITED STATES PATENT OFFICE.

ARCHIBALD J. MACDOUGALL, OF TORONTO, ONTARIO, CANADA, ASSIGNOR, BY DIRECT AND MESNE ASSIGNMENTS, OF ONE-SIXTH TO HERBERT C. BUGBIRD, OF NEW YORK, N. Y., ONE-SIXTH TO JAMES G. ROWE AND ONE-HALF TO RAY H. BENNETT, BOTH OF NORTH TONAWANDA, NEW YORK.

## PROCESS OF PRODUCING FERROUS OXID.

1,367,409.

Specification of Letters Patent.

Patented Feb. 1, 1921.

No Drawing.

Application filed August 21, 1920. Serial No. 405,055.

To all whom it may concern:

Be it known that I, ARCHIBALD J. MACDOUGALL, a subject of George V, King of the United Kingdom of Great Britain and 5 Ireland, residing at Toronto, in the Province of Ontario and Dominion of Canada, have invented certain new and useful Improvements in Processes of Producing Ferrous Oxid; and I do hereby declare the following 10 to be a full, clear, and exact description of the invention, such as will enable others skilled in the art to which it appertains to make and use the same.

My invention relates to the manufacture 15 of ferrous oxid by an electrolytic process.

At present it is customary to produce ferrous oxid by treating iron with sulfuric acid to obtain a sulfate of iron solution. This solution is then concentrated by evaporation 20 and crystallized. The crystals are subsequently calcined, thus producing ferric oxid, which latter is then reduced by hydrogen to form the ferrous oxid. This well known process not only necessitates the use 25 of sulfuric acid, an alkali and hydrogen, but it also involves five distinct operations, namely, the formation of the sulfate of iron, the evaporation of the sulfate solution, the crystallization, the calcining to produce 30 the ferric oxid, and the reduction of the oxid to the ferrous form by the use of hydrogen; and in addition the present process of manufacture has the disadvantage of often producing a product which is not 35 entirely ferrous oxid but contains some iron. Moreover, the apparatus required in making the sulfate of iron solution and in concentrating it and effecting crystallization has to be replaced frequently because of 40 rapid deterioration due to the action of the acid thereon; and a further disadvantage of the process at present followed is that the reduction of the ferric oxid by hydrogen requires heat, and great care must be taken 45 with the product to prevent its oxidation in the air to the ferric state due to its pyrophoric condition. The apparatus required in the practice of my process is much 50 cheaper, simpler and more easily maintained than that now employed in the production 55 of ferrous oxid, the cost of making the product is less and liability of iron being produced along with the ferrous oxid is minimized.

My process consists in forming ferrous 55 oxid from iron in an electrolytic cell in which the iron that is to enter into the ferrous oxid constitutes the anode, the cathode being any conductor which is insoluble in the electrolyte, and the electrolyte being 60 an aqueous solution of a salt. The iron of the anode is replenished as may be necessary from time to time as the production of the oxid proceeds; the cathode is preferably 65 iron or may conveniently be made of carbon; and the electrolyte is preferably an aqueous solution of sodium chlorid or of sodium sulfate, the former being more advantageous on account of its low cost and because its solubility does not vary greatly 70 with heating and also because of its low resistivity.

When a direct current is passed through 75 the anode, electrolyte and cathode, the salt of the aqueous solution is broken up, releasing an acid at the anode and an alkali at the cathode. The released acid dissolves the anode into an iron salt and the alkali released at the cathode, acting on this salt, precipitates out ferrous oxid of iron from 80 said salt. The ferrous oxid is then removed from the cell.

After the ferrous oxid has been removed from the cell it is freed of its moisture content. This may conveniently be done by extracting a portion of the moisture by means 85 of a filter press and by drying the ferrous oxid cake from the press in the presence of an inert or a reducing gas, the latter being preferable because a slight amount of an 90 occluded reducing agent tends to prevent oxidation of the product from the ferrous to the ferric state, thus increasing the stability of the compound as placed upon the market. Excellent results are obtained in the drying 95 operation if the temperature of the reducing agent does not exceed 500° F.

Assuming that an aqueous solution of sodium chlorid is adopted for the electrolyte, the reactions occurring in the production of 100 the ferrous oxid within the cell are as follows:



105



The aqueous solution of sodium chlorid is

electrolyzed to sodium hydroxid, chlorin, and hydrogen. The chlorin liberated by the electrolysis combines with the iron of the anode and forms chlorid of iron which is in turn acted upon by the sodium hydroxid produced by the electrolytic action, thus producing ferrous oxid and sodium chlorid, the hydroxyl radical being broken up in the course of electrolysis. The ferrous oxid is the desired product. The sodium chlorid is again electrolyzed, the action of the aqueous salt being cyclic.

The hydrogen which bubbles up through the electrolyte agitates it so that the iron salt formed there is brought into contact with the sodium hydroxid produced at the cathode, the result being that the reaction between the iron salt and the sodium hydroxid takes place readily and rapidly. If desired the hydrogen given off may be collected and used as a reducing gas in the drying of the ferrous oxid.

While in the example given sodium chlorid is the salt employed, it has been found that other soluble salts, particularly those of the so-called alkali metals, are applicable.

I claim:—

1. The process of producing ferrous oxid which consists in subjecting iron to the reaction in a cell of the products of the electrolysis of an electrolyte containing an aqueous solution of a salt.

2. The process of producing ferrous oxid which consists in forming an iron salt by subjecting iron within a cell to the acid product of the electrolysis of an aqueous solution of a salt, and converting said iron salt to ferrous oxid by the action of the alkaline product of the electrolysis of the said aqueous solution.

3. The process of producing ferrous oxid which consists in electrolyzing an aqueous solution of a salt in the presence of an iron anode and a cathode which is insoluble in said aqueous solution.

4. The process of producing ferrous oxid which consists in subjecting iron to the reaction in a cell of the products of the electrolysis of an aqueous solution of a salt, and subsequently drying said ferrous oxid in the presence of a reducing gas.

5. The process of producing ferrous oxid which consists in subjecting iron to the reaction in a cell of the products of the electrolysis of an aqueous solution of a sodium salt.

6. The process of producing ferrous oxid which consists in subjecting iron to the reaction in a cell of the products of the electrolysis of an aqueous solution of sodium chlorid.

7. The process of producing ferrous oxid which consists in electrolyzing an aqueous solution of a sodium salt in the presence of an iron anode and a cathode which is insoluble in said aqueous solution.

8. The process of producing ferrous oxid which consists in electrolyzing an aqueous solution of sodium chlorid in the presence of an iron anode and an iron cathode.

9. The process of producing ferrous oxid which consists in subjecting iron to the reaction in a cell of the products of the electrolysis of an aqueous solution of a salt, and subsequently drying said ferrous oxid in the presence of hydrogen.

10. The process of producing ferrous oxid which consists in electrolyzing an aqueous solution of sodium chlorid in the presence of an iron anode and an iron cathode, and subsequently drying said ferrous oxid in the presence of hydrogen.

11. The process of producing ferrous oxid which consists in subjecting iron to the reaction in a cell of the products of electrolysis of an aqueous solution of a salt of an alkaline substance.

12. The process of producing ferrous oxid which consists in subjecting iron to the reaction in a cell of the products of the electrolysis of an aqueous solution of a salt, said solution containing a salt of an inorganic acid dissolved therein.

13. The process of producing ferrous oxid which consists in forming an iron salt by subjecting iron within a cell to the acid product of the electrolysis of an aqueous solution of a salt of an inorganic acid and converting said iron salt to ferrous oxid by the action of the alkaline product of the electrolysis of said aqueous solution.

In testimony whereof I affix my signature.  
ARCHIBALD J. MACDOUGALL.